

Dec. 21, 1948.

E. B. KNOTT ET AL  
PHOTOGRAPHIC PROCESSES AND LIGHT-SENSITIVE  
ELEMENTS THEREFOR  
Filed Aug. 1, 1947

2,456,956



Patented Dec. 21, 1948

2,456,956

# UNITED STATES PATENT OFFICE

2,456,956

## PHOTOGRAPHIC PROCESSES AND LIGHT- SENSITIVE ELEMENTS THEREFOR

Edward Bowes Knott and Guy William Willis  
Stevens, Harrow, Wealdstone, England, assign-  
ors to Eastman Kodak Company, Rochester,  
N. Y., a corporation of New Jersey

Application August 1, 1947, Serial No. 765,636  
In Great Britain February 9, 1942

11 Claims. (Cl. 95-2)

1

This invention relates to photographic processes and materials therefor.

Various proposals have been made in the past for selectively processing inseparably superposed sensitive silver salt emulsion layers and sensitive silver salt emulsions mixed in a single layer. Such selective processings have been proposed for various purposes such as for multi-colour photography or for making numbers of prints of the same contrast from negatives of widely differing contrasts.

As is known the latent photographic image formed by the action of light on a photographic silver halide emulsion is not confined to the surface of the silver halide grains but it appears to be also distributed internally throughout those grains. It is possible to develop only the so-called surface latent image by means of developers which have little or no solvent action for the silver halide. One of us has described in the literature given below that after removal of the surface latent image the internal latent image can be developed as simply and conveniently as can an ordinary surface latent image if this is done by employing a developer having a solvent action for silver halide; moreover, the image so obtained indicated that the speed of the emulsion as measured by the internal image is often comparable with the speed as measured by the surface developed image. Such a developer is for convenience called an "internal" developer, and methods of development of internal latent images and solutions therefor are described in the Phot. J., 1942, 82, 42.

There is a type of emulsion, which while known per se, is according to our recent investigations of such a nature that the latent image is formed mostly inside the silver halide grains and there is relatively little surface latent image formed; such emulsions have not found much commercial use, in fact they have for a long time been considered as practically useless. We have found that such emulsions can have a considerable commercial use if they are developed with an internal developer, since in that case their effective practical speed as measured by the production of adequate densities is many times greater than was hitherto suspected. An example of such type of emulsion is that known as Burton's Emulsion given in Wall's "Photographic Emulsions" (1929) pp. 52-53. Moreover this type of emulsion may be prepared in other known manners, for instance by taking an ordinary silver bromide or an ordinary silver iodobromide emulsion containing between 0.5 and 5% silver iodide (based on the total silver halide), and coating it as a layer and then after drying, treating it with the following bath:

|                      |       |      |
|----------------------|-------|------|
| Potassium bichromate | grams | 12   |
| Conc. sulphuric acid | ccs.  | 12   |
| Water                | ccs.  | 1000 |

2

The time of treatment must be sufficient to inhibit surface latent image formation as much as possible as can easily be ascertained by exposing (after washing) and then treating with developers of Formulae I and III given below. Such an emulsion layer can then be used as it is or may be remelted and coated again as desired. These emulsions are examples of the type hereinafter referred to as Type I.

10 In the present invention we apply the aforesaid discovery to give a very advantageous method of achieving selective development of latent images in closely adjacent emulsions, especially of mixed emulsions, by employing for 15 one of the emulsions an emulsion which upon exposure forms the latent image mostly inside the grains according to Type I (as hereinafter defined) and for another emulsion, one which upon exposure forms surface latent image on the 20 grains according to Type II (as hereinafter defined) and differentially developing such latent images. Developers for developing such latent images are as follows:

### FORMULA I

25 "SURFACE" DEVELOPER

|                           |       |      |
|---------------------------|-------|------|
| p-Hydroxyphenylglycine    | grams | 10   |
| Sodium carbonate (cryst.) | do    | 100  |
| Water to                  | ccs.  | 1000 |

30 Development time 4 minutes at 20° C.

### FORMULA II(a)

#### "INTERNAL" DEVELOPER

|                                 |       |      |
|---------------------------------|-------|------|
| 35 Hydroquinone                 | grams | 15   |
| N-methyl-p-aminophenol sulphate | do    | 15   |
| Sodium sulphite, anhy.          | do    | 50   |
| Potassium bromide               | do    | 10   |
| Sodium hydroxide                | do    | 25   |
| 40 Sodium thiosulphate (cryst.) | do    | 20   |
| Water to                        | ccs.  | 1000 |

Development time 3 minutes at 20° C.

### FORMULA II(b)

#### "INTERNAL" DEVELOPER

|                                 |       |      |
|---------------------------------|-------|------|
| 45 Hydroquinone                 | grams | 12   |
| N-methyl-p-aminophenol sulphate | do    | 3    |
| Sodium sulphite (cryst.)        | do    | 90   |
| Potassium bromide               | do    | 4    |
| Sodium carbonate (cryst.)       | do    | 150  |
| 50 Sodium thiosulphate (cryst.) | do    | 20   |
| Water to                        | ccs.  | 1000 |

Development time 4 minutes at 20° C.

### FORMULA III

#### COMMERCIAL DEVELOPER

This is the same as Formula II(b) but omitting the sodium thiosulphate.

Formula II (a) is a more energetic developer than Formula II(b) so that it usually gives a

higher effective speed and a higher contrast than Formula II(b) but is often not so convenient since it has a higher tendency to aerial oxidation and to give fog.

While in this specification we have described our invention partly in regard to a theory of internal and surface latent images, the correctness or otherwise of such theory, is not essential to the successful working of the invention, it being only necessary to choose the emulsions according to the tests hereinafter given.

The present invention employs the following types of emulsions:

#### TYPE I

These are the emulsions which will develop (after exposure) in internal developers of the kind given in at least one of the Formulae II(a) and II(b), but will not develop or only slightly develop in Formula III or in Formula I.

##### (1) Normal Range of Exposures

As measured according to normal photographic testing technique, when a test layer of the emulsion is coated on a transparent support, for example glass, and the layer is exposed to an intensity scale, the whole of which is exposed for some fixed time between  $1/100$  and 1 second and is developed in the internal developer Formula II(a), the transmitted density obtained at any point along the  $\log_{10}E$  axis over a density range of 3.0 starting from the threshold of the curve ( $D=0.1$  above fog), should be at least 5 times, and preferably at least 10 times the transmitted density obtained when an identical test layer of the emulsion is developed with the surface developer of Formula I or preferably III, the measurements being made at the corresponding (i.e. same) points on the  $\log_{10}E$  axis; as indicated, the best (i.e. preferred) emulsions are those giving the highest density ratios and the very best (i.e. most preferred) emulsions can be selected with greater certainty by substituting Formula II (b) for II (a).

##### (2) Small Range of Exposures

For this purpose the emulsion need not conform to such a rigid requirement, for instance for making a tone correcting mask, but it is sufficient if in the above test the upper limit of 3.1 is substituted by an upper limit of 1.0.

#### TYPE II

These are the emulsions which when exposed to a light intensity scale, the whole of which is exposed for some fixed time between  $1/100$  and 1 second, will develop normally in Formulae I and III as well as in Formulae II(a) and II(b). As measured according to normal photographic testing technique, when a test layer of the emulsion is coated on a transparent support (e.g. glass) and the layer is exposed to a light intensity scale the whole of which is exposed for some fixed time between  $1/100$  and 1 second and is developed in the internal developer II(b), the transmitted density obtained at any point along the  $\log_{10}E$  axis of the curve between the density range of 0 to 3.0, preferably 0 to 2.0, does not exceed the transmitted density obtained when an identical test layer of the emulsion is developed in Formula III, the measurements of density being made at the same points on the  $\log_{10}E$  axis of the curve. Most known sensitive materials comprising a gelatino silver halide emulsion fall in the category of Type II.

Since Formula III contains sodium sulphite and Formula I is free from sulphite, and sulphite

is known to have some solvent action on silver chloride and bromide (although very little on silver iodide), it is apparent that when making any of the above measurements on an emulsion to obtain, with a high degree of precision, information on the amount of surface latent image given by such emulsion, it is important to use Formula I. As will be apparent hereinafter, in performing the invention a small amount of development of the internal latent image is of no real consequence for practical purposes, it may be advisable to employ Formula III, since this developer is not only less liable to aerial oxidation but gives better density in the image produced by the development of the Type II emulsion.

It is to be noted that an "internal" developer is necessarily capable of developing not only a latent image inside grains but also of developing a latent image on the surface of grains (whether such grains contain internal latent image or not) and also of carrying on the development of a surface latent image which has previously been only partly developed.

It is also to be noted that where a "surface" developer is employed to develop a surface latent image, then all grains which are thereby fully developed cannot be subsequently developed at all in an "internal" developer.

According to one feature of the present invention there is provided the method of selectively producing images in a photographic material comprising silver salt emulsions on a single support which comprises employing therefor two emulsions one of which is Type I as herein defined and the other of which is of Type II as herein defined, selectively exposing (simultaneously or consecutively) both emulsions to form latent images therein and differentially developing the latent images so formed.

In this form of the invention the differential development may be performed by treating the whole material in a developer which develops practically only surface latent image (preferably to completion) and then treating the whole material with a developer which develops internal latent image.

The present invention also provides a useful sensitive photographic material comprising on a single support two sensitive silver salt emulsions one of which upon exposure forms the latent image mostly inside the grains as defined by Type I above and the other of which upon exposure forms a surface latent image as defined by Type II above, the combination being such that each of such emulsions can be selectively exposed.

According to a modification of the invention there is provided the method of producing a number of prints of differing gradations (gammas) wherein each of the prints is made by exposure of a sensitive material comprising on a single support two silver salt emulsions giving different gammas, one of which is of Type I as herein defined and the other of which is of Type II as herein defined and the latent images so formed in the various prints are developed in such wise that the emulsions of Type I and II are differentially developed from print to print.

The invention also provides the method of producing a photographic image of a predetermined contrast wherein such image is formed by exposure of a sensitive material comprising on a single support two silver salt emulsions giving differing gammas, one of which is of Type I as herein defined and the other of which is of Type II as herein defined, and the material is developed

in a developer whose capabilities of developing internal and surface latent image are so related as to give the said contrast.

The invention includes a sensitive material for this purpose and comprising on a single support, two sensitive silver salt emulsions, either as superimposed or side by side layers or mixed, one of which is of Type I (as herein defined) and upon development thereof gives an image of one gamma and the other of which is of Type II (as herein defined) and upon development thereof gives an image of a different gamma.

For some purposes such a sensitive material is useful for producing two photographic images on a single support by exposing the material and then after treating the whole material in a developer which develops practically only the surface latent image or images, the whole material is treated with a developer which develops the internal latent image.

Whenever it is desired that several emulsions on the same support can each be selectively exposed, (i. e. simultaneously or consecutively) this can be done by several known methods, for instance,

(a) Making the emulsions differentially colour sensitive,

(b) If the emulsions are in superimposed layers, placing a light absorbing filter layer between them or in one of them such as in the Type I emulsion,

(c) If the emulsions are side by side (i. e. in different areas of the support) they can be easily exposed separately.

Possible ways of arranging an emulsion of Type I and an emulsion of Type II in the present invention are illustrated by the following:

(1) A not specially colour sensitised emulsion of Type I having a relatively high blue sensitivity mixed with or superimposed on a green or red sensitised emulsion of Type II of relatively low blue sensitivity.

(2) A green sensitive emulsion of Type I mixed or superimposed on a red sensitive emulsion of Type II.

(3) A not specially colour sensitised emulsion of Type I coated on a not specially colour sensitised emulsion of Type II with a blue absorbing filter layer therebetween, or the filtering material may be in one of the emulsions such as in the Type I emulsion. Such emulsions can be on the same side or opposite sides of the support.

(4) A Type I emulsion, colour sensitised or not, and a Type II emulsion, colour sensitised or not, coated side by side (i. e. in different areas of the support).

The invention is not limited to these specific ways which are given by way of example only.

We have found that a useful multi-colour photographic process and sensitive material for use therein results if there is employed on a single support two emulsions respectively of Types I and II, the combination being such that they are effectively differentially colour sensitive.

The following Example I illustrates a material which can be employed as a two-colour element in a three-colour process.

#### EXAMPLE I

To 3,500 ccs. of an emulsion of Type I (which has not been specially colour sensitised) containing the silver halide equivalent of 200 grams of silver nitrate there is added 200 ccs. of an 8% alcoholic solution of hydrolysed soft lac resin (for such resins see U. S. Patent No. 2,199,978). To 300 ccs. of a Type II silver chloride emul-

sion containing the silver chloride equivalent to 60 grams of silver nitrate and sensitised to green by addition of 175 ccs. of a 0.02% alcoholic solution of the dye 5-[2-ethyl-1(2-benzoxazolylidene)ethylidene]-3-n-heptyl-1-phenyl-2-thiodihydantoin (Example 3 of U. S. Patent No. 2,282,116) there is added 60 ccs. of an 8% of alcoholic solution of the said hydrolysed soft lac resin. The two emulsions are then mixed at 30° C. and coated on a support such as paper, or they may be coated as superimposed layers. After exposure to a colour image or object this material can be processed to give a two-colour negative image by treating it as follows:

(1) Treat in an ordinary surface colour developer containing a colour coupler which gives a magenta coloured image, for a time sufficient to colour develop the surface latent image in the Type II emulsion.

(2) After washing, develop in a developer containing a coupler giving an orange coloured image such developer containing also a silver halide solvent, such as 5 to 40 grams per litre of sodium thiosulphate, so as to develop the internal latent image in the Type I emulsion.

(3) After washing dissolve out all silver formed and all unused silver halides in a bath of sodium thiosulphate and potassium ferricyanide.

This example could obviously be applied to the processing of a two-colour element in a two-colour process if the coupler which gives magenta is replaced by one giving blue-green.

Selective developability depending on latent image distribution may also be usefully combined with known means (see for example U. S. Patent Nos. 2,231,684 and 2,226,639) for obtaining selective developability. For instance in a subtractive process of three-colour photography, silver bromide or iodo-bromide emulsion of Type II may be mixed with a silver bromide or iodo-bromide emulsion of Type I and a silver chloride emulsion of Type II; alternatively, these emulsions may be coated in three superimposed layers or in two superimposed layers one of which consists of a mixture of two of the emulsions. After exposure of such material the silver chloride emulsion may be selectively developed before the other emulsions are separately developed in accordance with their type. Of course, any two superimposed emulsion layers both of the same type can be selectively processed in known manner, such as by employing loaded developing solutions as described in U. S. Patent No. 2,059,884, a third emulsion of the other type being mixed in one of such layers.

Protective layers which are only penetrated by suitable acid or alkaline solutions may also be used in the same way.

The following illustrates a three-colour process:

#### EXAMPLE II

On a support, there is first coated a silver bromide or iodo-bromide emulsion of Type II sensitised to the red with, for instance, 3,3'-dimethyl-4:5:4':5'-dibenzthiacarbocyanine iodide. Over the layer so formed there is coated a mixture of a silver chloride emulsion (Type II) sensitised to the green with a sensitising dye having little or no tendency to wander (e. g. the aforementioned dye of Example 3 of U. S. Patent No. 2,282,116) and an emulsion of Type I of silver iodo-bromide sensitive only to the blue. This Type I emulsion is one which absorbs blue light very strongly and this has the effect of reducing

considerably the effective blue sensitivity of the red sensitive layer. The blue sensitivity of the silver chloride emulsion is so low that there is practically no image formed therein when the blue sensitive emulsion mixed therewith is properly exposed. This mixture may be made exactly as the mixture prescribed in Example I. The two emulsions of the mixture may if desired be coated on superimposed layers. Alternatively, the blue sensitive emulsion can be coated by itself as a layer over a layer consisting of a mixture of the red and green sensitive emulsions and the blue sensitivity of the latter can be effectively reduced in known manner by interposing a yellow filter layer between the layers as described in British Patent No. 500,611.

After exposure of the material to a coloured object or image, it is processed as follows:

(1) Treat in a mildly acting first developer containing a colour coupler which gives a magenta coloured image, for a time just sufficient to colour develop the surface latent image in the silver chloride emulsion without having any practical effect on the silver bromide (see for instance U. S. Patents Nos. 2,226,639 and 2,231,684).

The mildly acting first developer just referred to is composed as follows:

|                                    |        |    |
|------------------------------------|--------|----|
| Water                              | liters | 1  |
| Diethyl para-phenylene diamine     |        |    |
| HCl                                | grams  | 10 |
| Sodium sulphite                    | do     | 5  |
| Sodium carbonate                   | do     | 20 |
| Potassium bromide (Molar solution) | ccs    | 2  |

with the addition of the coupler.

(2) After washing, develop in a surface developer containing a coupler giving a blue-green coloured image for sufficient time to develop only but completely the surface latent image in the lower red sensitive emulsion layer (Type II emulsion).

(3) After again washing, develop in a developer containing a coupler giving a yellow coloured image, such developer containing also a silver solvent, such as 5 to 40 grams per liter of sodium thiosulphate, so as to develop the internal latent image in the silver bromide or iodo-bromide emulsion (Type I) in the upper layer.

(4) After washing dissolve out all silver formed and all unused silver halides in a bath of sodium thiosulphate and potassium ferricyanide.

A less advantageous form of the invention is illustrated by the following example:

### EXAMPLE III

A film support is coated with a high contrast fine grain process type emulsion, having a silver halide to gelatin ratio of 0.7:1, at a rate to give 0.5 grain of silver per square foot. The layer is hardened fully in known manner sufficient to make the layer able to withstand the bleaching bath given below. After drying, the layer is treated for 3 hours at 70° F. in the following solution:

|                        |       |      |
|------------------------|-------|------|
| Potassium dichromate   | grams | 12   |
| Sulphuric acid (conc.) | ccs   | 12   |
| Water to make          | ccs   | 1000 |

It is then washed for 5 minutes in running water, and then treated for 2 minutes at 70° F. in:

|                    |       |      |
|--------------------|-------|------|
| Sodium bicarbonate | grams | 50   |
| Water to make      | ccs   | 1000 |

a final thirty minutes washing is then given and the layer is dried.

This treatment converts the process emulsion from Type II to Type I. The other side of the film is then successively coated with a blue absorbing filter layer and then an emulsion of Type II. This material can be used in a two colour process as a printing material where it is desired to expose both emulsions prior to any processing step.

Other examples of the use and selective treatment of emulsions of different types on a single support are as follows; and in these examples the emulsions may be also differentially colour sensitised so that they can be exposed selectively by different coloured lights.

(a) Side by side stereoscopic images (i. e. on different areas of the support) produced on the same cinematograph film which are to be developed to red and green respectively (for viewing through red and green spectacles) may be processed in a simple manner by treatment of the whole film first with a developing solution for developing only one of the emulsions and subsequently with a developing solution for developing the other emulsion.

(b) A picture image and a sound track image side by side on the same support can be developed separately for instance to different gammas, without the trouble of applying the development solutions to the separate picture and sound areas of the cinematograph film (e. g. by applicator rollers) by employing (e. g. in admixture) an emulsion of one type for printing the sound track and an emulsion or emulsions of the other type for printing the picture.

(c) Where it may be desirable to develop the two longitudinal halves of 16 mm. film separately, for example, one half to black and white and the other half to a coloured image for any purpose; this can be done by adopting a procedure analogous to that indicated in (a) and (b).

Although the invention which has been described in detail above requires that the emulsions of Types I and II should be so constituted or arranged that either of them can be selectively exposed, it is possible as has already been indicated to modify the invention by dispensing with this requirement and making the emulsions of the said two types so that they give different gammas and then such a material, although less useful than those previously described, can be used for so-called multi-contrast purposes, such as for producing images of different contrasts from negatives of the same contrast or images of the same contrast from negatives of different contrasts; for such purposes it is usually desirable that the gammas should differ by at least 2.5, and the low gamma being not more than 1.8, such gammas being measured as set forth in British Patent No. 541,510, it being understood that the appropriate developers of Formula II(b) and III are used for developing the Type I and Type II emulsions respectively.

The emulsions can be dye-sensitised or not. As an example we can employ an emulsion of Type II giving a low gradation in Formula III and an emulsion of Type I giving a high gradation in Formula II(b). In this combination the threshold speed of Type II emulsion when developed in developer Formula II or III should for example be higher than that of Type I emulsion when developed in developer Formula II(b) preferably the characteristic curves under these conditions should cross at about a density of one. The emulsion giving the higher gradation (gamma) can be made as the emulsion described

in Example III herein; preferably the fine grain process type emulsion used should be one of good uniform grain size and giving a gamma of about 4. The other emulsion can be one of Type II giving a gradation of 1.2.

The material so made can be printed with white light and then the contrast of the image controlled by choice of the developer. For example, using an emulsion of Type II giving a low gradation in Formula III and an emulsion of Type I giving a high gradation in Formula II(b) and still higher in Formula II(a), the image will be of relatively low contrast if developed in a developer such as Formula III, of relatively medium contrast in a developer of Formula II(b) or a higher contrast in Formula II(a). Using either Formula II(a) or II(b) a higher contrast can be obtained if before development the exposed material is first treated in a mild silver oxidising bath which destroys the surface latent image in the emulsion of Type II.

Two examples of such solutions are the following solutions A and B.

*Solution A*

|                        |       |      |
|------------------------|-------|------|
| Potassium ferricyanide | grams | 20   |
| Potassium bromide      | do    | 10   |
| Water to               | ccs   | 1000 |

*Solution B*

|                      |       |      |
|----------------------|-------|------|
| Potassium dichromate | grams | 2    |
| Conc. sulphuric acid | ccs   | 2    |
| Water to             | ccs   | 1000 |

As another example, the threshold speed of the Type II emulsion can be equal to or lower than that of the Type I emulsion. Such a material gives low contrast mainly due to the Type II emulsion on development in Formula III and a high contrast mainly due to the Type I emulsion on development in Formula II(a) or II(b).

As has previously been indicated material of this kind employing emulsions of Types I and II having different gammas may be processed also by treating the whole material after exposure in a developer which develops practically only the surface latent image or images, and thereafter treating the whole material in a developer which develops the internal latent image.

This application is a continuation in part of our co-pending application Serial No. 528,738, filed March 30, 1944, now abandoned.

The accompanying drawing is a flow-diagram of one embodiment of our invention and shows the operation of the process. At B is shown a support coated with a layer of a low gradation (contrast) emulsion which forms latent image on the surface of the silver halide grains and has a threshold speed equal to or lower than the threshold speed of a second layer of emulsion coated upon the low gradation emulsion layer, said second emulsion layer consisting of a high gradation emulsion which forms the latent image mostly inside the silver halide grains. Upon exposing this photographic element to the lighted object shown at A, a negative latent image is formed in both emulsion layers as shown at C. Upon developing the exposed photographic element shown at C in a developer which develops substantially only surface latent image, the latent image in the lower emulsion layer is developed to a negative image of low contrast while the negative latent image in the upper layer is substantially unaffected as shown at D. At this point, the photographic element shown at D can be fixed and washed, or the element can be developed

in a developer which develops internal latent image, whereupon the negative latent image in the upper emulsion layer is also developed giving a negative image of high contrast as shown at E.

5 The exposed photographic element shown at C, if developed in a developer which develops internal latent image, gives a negative image in both emulsion layers, the overall image being of high contrast as shown at F.

10 What we claim as our invention and desire to be secured by Letters Patent of the United States is:

1. A method of selectively producing photographic images in a photographic element containing, inseparably combined and extending over

15 the same area on a single support, a light-sensitive silver salt photographic emulsion (I) a test layer of which coated on a transparent support and the layer exposed to a light intensity scale for a fixed time between  $\frac{1}{100}$  and 1 second and development for 3 minutes at 20° C. in the following developer (IIa):

|                                 |       |      |
|---------------------------------|-------|------|
| Hydroquinone                    | grams | 15   |
| N-methyl-p-aminophenol sulphate | do    | 15   |
| Sodium sulphite, anhydrous      | do    | 50   |
| Potassium bromide               | do    | 10   |
| Sodium hydroxide                | do    | 25   |
| Sodium thiosulphate, crystals   | do    | 20   |
| Water to                        | ccs   | 1000 |

30 gives a transmitted density at any point along the  $\log_{10}E$  axis over a density range of 3.0 starting from the threshold of the characteristic curve beginning at a density of 0.1 above fog, at least 5 times the transmitted density obtained when an identical test layer of the emulsion is developed for 4 minutes at 20° C. in the following developer (I):

|                            |       |      |
|----------------------------|-------|------|
| p-hydroxyphenylglycine     | grams | 10   |
| Sodium carbonate, crystals | do    | 100  |
| Water to                   | ccs   | 1000 |

the measurements of density being made at the same points on the  $\log_{10}E$  axis, and another light sensitive silver salt photographic emulsion (II) a test layer of which coated on a transparent support and the layer exposed to a light intensity scale for a fixed time between  $\frac{1}{100}$  and 1 second and development for 4 minutes at 20° C. in the following developer (IIb):

|                                  |       |      |
|----------------------------------|-------|------|
| 50 Hydroquinone                  | grams | 12   |
| N-methyl-p-aminophenol sulphate  | do    | 3    |
| Sodium sulphite, crystals        | do    | 90   |
| Potassium bromide                | do    | 4    |
| Sodium carbonate, crystals       | do    | 150  |
| 55 Sodium thiosulphate, crystals | do    | 20   |
| Water to                         | ccs   | 1000 |

gives a transmitted density between the range of 0 to 2.0 which does not exceed the transmitted density obtained when an identical test layer of the emulsion (II) is developed for 4 minutes at 20° C. in the following developer (III):

|                                 |       |      |
|---------------------------------|-------|------|
| Hydroquinone                    | grams | 12   |
| N-methyl-p-aminophenol sulphate | do    | 3    |
| 65 Sodium sulphite, crystals    | do    | 90   |
| Potassium bromide               | do    | 4    |
| Sodium carbonate, crystals      | do    | 150  |
| Water to                        | ccs   | 1000 |

70 comprising exposing each emulsion to light, then treating the whole element with a developer which develops substantially only the latent image which is developable by developer (III) and then developing the whole element in a developer which develops the latent image which is developable in developer (IIa).

2. A method of selectively producing photographic images in a photographic element containing, inseparably combined and extending over the same area on a single support, a light sensitive silver halide emulsion (I) a test layer of which coated on a transparent support and the layer exposed to a light intensity scale, for a fixed time between  $\frac{1}{100}$  and 1 second and development for 3 minutes at 20° C. in the following developer (IIa):

|                                 |       |      |
|---------------------------------|-------|------|
| Hydroquinone                    | grams | 15   |
| N-methyl-p-aminophenol sulphate | do    | 15   |
| Sodium sulphite, anhydrous      | do    | 50   |
| Potassium bromide               | do    | 10   |
| Sodium hydroxide                | do    | 25   |
| Sodium thiosulphate, crystals   | do    | 20   |
| Water to                        | ccs   | 1000 |

gives a transmitted density at any point along the  $\log_{10}E$  axis over a density range of 3.0 starting from the threshold of the characteristic curve beginning at a density of 0.10 above fog, at least 5 times the transmitted density obtained when an identical test layer emulsion is developed for 4 minutes at 20° C. in the following developer (I):

|                            |       |      |
|----------------------------|-------|------|
| p-Hydroxyphenylglycine     | grams | 10   |
| Sodium carbonate, crystals | do    | 100  |
| Water to                   | ccs   | 1000 |

the measurements being made at the same points on the  $\log_{10}E$  axis, and another light sensitive silver halide photographic emulsion (II) a test layer of which coated on a transparent support and the layer is exposed to a light intensity scale, for a fixed time between  $\frac{1}{100}$  and 1 second and development for 4 minutes at 20° C. in the following developer (IIb):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs   | 1000 |

gives a transmitted density between the range of 0 to 2.0 which does not exceed the transmitted density obtained when an identical test layer of the emulsion (II) is developed for 4 minutes at 20° C. in the following developer (III).

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Water to                        | ccs   | 1000 |

comprising exposing each emulsion to light, then treating the whole element with a developer which develops substantially only the latent image which is developable by developer (III) and then developing the whole element in a developer which develops the latent image which is developable in developer (IIa).

3. A method of selectively producing photographic images in a photographic element containing, inseparably combined and extending over the same area on a single support, a light-sensitive silver halide emulsion (I) a test layer of which coated on a transparent support and the layer exposed to a light intensity scale for a fixed time between  $\frac{1}{100}$  and 1 second and de-

velopment for 3 minutes at 20° C. in the following developer (IIa):

|                                 |       |      |
|---------------------------------|-------|------|
| Hydroquinone                    | grams | 15   |
| N-methyl-p-aminophenol sulphate | do    | 15   |
| Sodium sulphite, anhydrous      | do    | 50   |
| Potassium bromide               | do    | 10   |
| Sodium hydroxide                | do    | 25   |
| Sodium thiosulphate, crystals   | do    | 20   |
| Water to                        | ccs   | 1000 |

10 gives a transmitted density at any point along the  $\log_{10}E$  axis over a density range of 3.0 starting from the threshold of the characteristic curve beginning at a density of 0.1 above fog, at least 10 times the transmitted density obtained when an identical test layer of the emulsion is developed for 4 minutes at 20° C. in the following developer (I):

|                            |       |      |
|----------------------------|-------|------|
| p-Hydroxyphenylglycine     | grams | 10   |
| Sodium carbonate, crystals | do    | 100  |
| Water to                   | ccs   | 1000 |

20 the measurements being made at the same points on the  $\log_{10}E$  axis, and another light sensitive silver halide photographic emulsion (II) a test layer of which coated on a transparent support and the layer exposed to a light intensity scale for a fixed time between  $\frac{1}{100}$  and 1 second and development for 4 minutes at 20° C. in the following developer (IIb):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs   | 1000 |

30 gives a transmitted density between the range of 0 to 2.0 which does not exceed the transmitted density obtained when an identical test layer of the emulsion (II) is developed for 4 minutes at 20° C. in the following developer (III):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Water to                        | ccs   | 1000 |

40 comprising exposing each emulsion to light, then treating the whole element with a developer which develops substantially only the latent image which is developable by developer (III) and then developing the whole element in a developer which develops the latent image which is developable in developer (IIa).

45 4. A method of selectively producing photographic images in a photographic element containing, inseparably combined and extending over the same area on a single support, a light sensitive silver halide emulsion (I) a test layer of which coated on a transparent support and the layer exposed to a light intensity scale for a fixed time between  $\frac{1}{100}$  and 1 second and development for 4 minutes at 20° C. in the following developer (IIb):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs   | 1000 |

50 50 gives a transmitted density at any point along the  $\log_{10}E$  axis over a density range of 3.0 start-

ing from the threshold of the characteristic curve beginning at a density of 0.1 above fog, at least 10 times the transmitted density obtained when an identical test layer of the emulsion is developed for 4 minutes at 20° C. in the following developer (III):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Water to                        | ccs   | 1000 |

the measurements being made at the same points on the  $\log_{10}E$  axis, and another light sensitive silver halide photographic emulsion (II) a test layer of which coated on a transparent support and the layer exposed to a light intensity scale for a fixed time between  $\frac{1}{100}$  and 1 second and development for 4 minutes at 20° C. in the aforesaid developer (IIb) gives a transmitted density between the range of 0 to 2.0, which does not exceed the transmitted density obtained when an identical test layer of the emulsion (II) is developed for 4 minutes at 20° C. in the aforesaid developer (III) comprising exposing each emulsion to light, then treating the whole element with a developer which develops substantially only the latent image which is developable by developer (III) and then developing the whole element in a developer which develops the latent image which is developable in developer (IIb).

5. A sensitive photographic element comprising, inseparably combined and extending over the same area on a single support, a light sensitive silver salt emulsion (I) a test layer of which coated on a transparent support and the layer exposed to a light intensity scale for a fixed time between  $\frac{1}{100}$  and 1 second and development for 3 minutes at 20° C. in the following developer (IIa):

|                                 |       |      |
|---------------------------------|-------|------|
| Hydroquinone                    | grams | 15   |
| N-methyl-p-aminophenol sulphate | do    | 15   |
| Sodium sulphite, anhydrous      | do    | 50   |
| Potassium bromide               | do    | 10   |
| Sodium hydroxide                | do    | 25   |
| Sodium thiosulphate, crystals   | do    | 20   |
| Water to                        | ccs   | 1000 |

gives a transmitted density at any point along the  $\log_{10}E$  axis over a density range of 3.0 starting from the threshold of the characteristic curve beginning at a density of 0.1 above fog, at least 5 times the transmitted density obtained when an identical test layer of the emulsion is developed for 4 minutes at 20° C. in the following developer (I):

|                            |       |      |
|----------------------------|-------|------|
| p-Hydroxyphenylglycine     | grams | 10   |
| Sodium carbonate, crystals | do    | 100  |
| Water to                   | ccs   | 1000 |

the measurements of density being made at the same points on the  $\log_{10}E$  axis, and another light sensitive silver salt photographic emulsion (II) a test layer of which coated on a transparent support and the layer exposed to a light intensity scale for a fixed time between  $\frac{1}{100}$  and 1 second and development for 4 minutes at 20° C. in the following developer (IIb):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs   | 1000 |

gives a transmitted density between the range of 0 to 2.0, which does not exceed the transmitted density obtained when an identical test layer of the emulsion (II) is developed for 4 minutes at 20° C. in the following developer (III):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Water to                        | ccs   | 1000 |

6. A sensitive photographic element comprising, inseparably combined and extending over the same area on a single support, a light sensitive silver halide emulsion (I), a test layer of which coated on a transparent support and the layer exposed to a light intensity scale for a fixed time between  $\frac{1}{100}$  and 1 second and development for 3 minutes at 20° C. in the following developer (IIa):

|                                 |       |      |
|---------------------------------|-------|------|
| Hydroquinone                    | grams | 15   |
| N-methyl-p-aminophenol sulphate | do    | 15   |
| Sodium sulphite, anhydrous      | do    | 50   |
| Potassium bromide               | do    | 10   |
| Sodium hydroxide                | do    | 25   |
| Sodium thiosulphate, crystals   | do    | 20   |
| Water to                        | ccs   | 1000 |

gives a transmitted density at any point along the  $\log_{10}E$  axis over a density range of 3.0 starting from the threshold of the characteristic curve beginning at a density of 0.1 above fog, at least 5 times the transmitted density obtained when an identical test layer of the emulsion is developed for 4 minutes at 20° C. in the following developer (I):

|                            |       |      |
|----------------------------|-------|------|
| p-Hydroxyphenylglycine     | grams | 10   |
| Sodium carbonate, crystals | do    | 100  |
| Water to                   | ccs   | 1000 |

the measurements of density being made at the same points on the  $\log_{10}E$  axis, and another light sensitive silver halide photographic emulsion (II) a test layer of which coated on a transparent support and the layer exposed to a light intensity scale for a fixed time between  $\frac{1}{100}$  and 1 second and development for 4 minutes at 20° C. in the following developer (IIb):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs   | 1000 |

gives a transmitted density between the range of 0 to 2.0, which does not exceed the transmitted density obtained when an identical test layer of the emulsion (II) is developed for 4 minutes at 20° C. in the following developer (III):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Water to                        | ccs   | 1000 |

7. A sensitive photographic element comprising, inseparably combined and extending over the same area on a single support, a light sensitive silver halide emulsion (I) a test layer of which coated on a transparent support and the layer exposed to a light intensity scale for a fixed time between  $\frac{1}{100}$  and 1 second and development for

3 minutes at 20° C. in the following developer (IIa):

|                                 |       |      |
|---------------------------------|-------|------|
| Hydroquinone                    | grams | 15   |
| N-methyl-p-aminophenol sulphate | do    | 15   |
| Sodium sulphite, anhydrous      | do    | 50   |
| Potassium bromide               | do    | 10   |
| Sodium hydroxide                | do    | 25   |
| Sodium thiosulphate, crystals   | do    | 20   |
| Water to                        | ccs.  | 1000 |

gives a transmitted density at any point along the  $\log_{10}E$  axis over a density range of 3.0 starting from the threshold of the characteristic curve beginning at a density of 0.1 above fog, at least 10 times the transmitted density obtained when an identical test layer of the emulsion is developed for 4 minutes at 20° C. in the following developer (I):

|                            |       |      |
|----------------------------|-------|------|
| p-Hydroxyphenylglycine     | grams | 10   |
| Sodium carbonate, crystals | do    | 100  |
| Water to                   | ccs.  | 1000 |

the measurements of density being made at the same points on the  $\log_{10}E$  axis, and another light sensitive silver halide photographic emulsion (II) a test layer of which coated on a transparent support and the layer exposed to a light intensity scale for a fixed time between  $1/100$  and 1 second and development for 4 minutes at 20° C. in the following developer (IIb):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs.  | 1000 |

gives a transmitted density between the range of 0 to 2.0, which does not exceed the transmitted density obtained when an identical test layer of the emulsion (II) is developed for 4 minutes at 20° C. in the following developer (III):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Water to                        | ccs.  | 1000 |

8. A sensitive photographic element comprising, inseparably combined and extending over the same area on a single support, a light sensitive silver halide emulsion (I) a test layer of which coated on a transparent support and the layer exposed to a light intensity scale for a fixed time between  $1/100$  and 1 second and development for 4 minutes at 20° C. in the following developer (IIb):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs.  | 1000 |

gives a transmitted density at any point along the  $\log_{10}E$  axis, over a density range of 3.0 starting from the threshold of the characteristic curve beginning at a density of 0.1 above fog, at least 10 times the transmitted density obtained when an identical test layer of the emulsion is de-

veloped for 4 minutes at 20° C. in the following developer (III):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Water to                        | ccs.  | 1000 |

the measurements being made at the same points on the  $\log_{10}E$  axis, and another light sensitive silver halide photographic emulsion (II) a test layer of which coated on a transparent support and the layer exposed to a light intensity scale for a fixed time between  $1/100$  and 1 second and development for 4 minutes at 20° C. in the aforesaid developer (IIb) gives a transmitted density between the range of 0 to 2.0 which does not exceed the transmitted density obtained when an identical test layer of the emulsion (II) is developed for 4 minutes at 20° C. in the aforesaid developer (III).

9. A sensitive photographic element comprising two inseparably superposed emulsion layers extending over the same area on a single support, one emulsion layer being a light sensitive silver halide photographic emulsion (I) a test layer of which coated on a transparent support and the layer exposed to a light intensity scale for a fixed time between  $1/100$  and 1 second and development for 3 minutes at 20° C. in the following developer (IIc):

|                                 |       |      |
|---------------------------------|-------|------|
| Hydroquinone                    | grams | 15   |
| N-methyl-p-aminophenol sulphate | do    | 15   |
| Sodium sulphite, anhydrous      | do    | 50   |
| Potassium bromide               | do    | 10   |
| Sodium hydroxide                | do    | 25   |
| Sodium thiosulphate, crystals   | do    | 20   |
| Water to                        | ccs.  | 1000 |

gives a transmitted density at any point along the  $\log_{10}E$  axis over a density range of 3.0 starting from the threshold of the characteristic curve beginning at a density of 0.1 above fog, at least 10 times the transmitted density obtained when an identical test layer of the emulsion is developed for 4 minutes at 20° C. in the following developer (I):

|                            |       |      |
|----------------------------|-------|------|
| p-Hydroxyphenylglycine     | grams | 10   |
| Sodium carbonate, crystals | do    | 100  |
| Water to                   | ccs.  | 1000 |

55. the measurements of density being made at the same points on the  $\log_{10}E$  axis, and the other emulsion layer being a light sensitive silver halide photographic emulsion (II) a test layer of which coated on a transparent support and the layer exposed to a light intensity scale for a fixed time between  $1/100$  and 1 second and development for 4 minutes at 20° C. in the following developer (IIb):

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs.  | 1000 |

gives a transmitted density below the range of 0 to 2.0, which does not exceed the transmitted density obtained when an identical test layer of

the emulsion (II) is developed for 4 minutes at 20° C. in the following developer (III) :

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Water to                        | ccs   | 1000 |

10. A sensitive photographic element comprising two inseparably superposed differentially color sensitive emulsion layers extending over the same area on a single support, one emulsion layer being a light sensitive silver halide photographic emulsion (I) a test layer of which coated on a transparent support and the layer exposed to a light intensity scale for a fixed time between  $1/100$  and 1 second and development for 3 minutes at 20° C. in the following developer (IIa) :

|                                 |       |      |
|---------------------------------|-------|------|
| Hydroquinone                    | grams | 15   |
| N-methyl-p-aminophenol sulphate | do    | 15   |
| Sodium sulphite, anhydrous      | do    | 50   |
| Potassium bromide               | do    | 10   |
| Sodium hydroxide                | do    | 25   |
| Sodium thiosulphate, crystals   | do    | 20   |
| Water to                        | ccs   | 1000 |

gives a transmitted density at any point along the  $\log_{10}E$  axis over a density range of 3.0 starting from the threshold of the characteristic curve beginning at a density of 0.1 above fog, at least 10 times the transmitted density obtained when an identical test layer of the emulsion is developed for 4 minutes at 20° C. in the following developer (I) :

|                            |       |      |
|----------------------------|-------|------|
| p-Hydroxyphenylglycine     | grams | 10   |
| Sodium carbonate, crystals | do    | 100  |
| Water to                   | ccs   | 1000 |

the measurements of density being made at the same points on the  $\log_{10}E$  axis, and the other emulsion layer being a light sensitive silver halide photographic emulsion (II) a test layer of which coated on a transparent support and the layer exposed to a light intensity scale for a fixed time between  $1/100$  and 1 second and development for 4 minutes at 20° C. in the following developer (IIb) :

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs   | 1000 |

gives a transmitted density between the range of 0 to 2.0, starting from the threshold of the characteristic curve beginning at a density of 0.1 above fog which does not exceed the transmitted density obtained when an identical test layer of the emulsion (II) is developed for 4 minutes at 20° C. in the following developer (III) :

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Water to                        | ccs   | 1000 |

11. A sensitive photographic element comprising three inseparably superposed differentially color sensitive emulsion layers, extending over the same area on a single support, one emulsion layer being a light sensitive silver halide photographic emulsion (I) a test layer of which coated on a transparent support and the layer exposed to a light intensity scale for a fixed time between  $1/100$  and 1 second and development for 3 minutes at 20° C. in the following developer (IIa) :

|                                 |       |      |
|---------------------------------|-------|------|
| Hydroquinone                    | grams | 15   |
| N-methyl-p-aminophenol sulphate | do    | 15   |
| Sodium sulphite, anhydrous      | do    | 50   |
| Potassium bromide               | do    | 10   |
| Sodium hydroxide                | do    | 25   |
| Sodium thiosulphate, crystals   | do    | 20   |
| Water to                        | ccs   | 1000 |

gives a transmitted density at any point along the  $\log_{10}E$  axis over a density range of 3.0 starting from the threshold of the characteristic curve beginning at a density of 0.1 above fog, at least 10 times the transmitted density obtained when an identical test layer of the emulsion is developed for 4 minutes at 20° C. in the following developer (I) :

|                            |       |      |
|----------------------------|-------|------|
| p-Hydroxyphenylglycine     | grams | 10   |
| Sodium carbonate, crystals | do    | 100  |
| Water to                   | ccs   | 1000 |

30 the measurements of density being made at the same points on the  $\log_{10}E$  axis, and the other two emulsion layers being each a light sensitive silver halide photographic emulsion (II) a test layer of which coated on a transparent support and the layer exposed to a light intensity scale for a fixed time between  $1/100$  and 1 second and development for 4 minutes at 20° C. in the following developer (IIb) :

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Sodium thiosulphate, crystals   | do    | 20   |
| Water to                        | ccs   | 1000 |

gives a transmitted density between the range of 0 to 2.0, which does not exceed the transmitted density obtained when an identical test layer of the emulsion (II) is developed for 4 minutes at 20° C. in the following developer (III) :

|                                 |       |      |
|---------------------------------|-------|------|
| Hydroquinone                    | grams | 12   |
| N-methyl-p-aminophenol sulphate | do    | 3    |
| Sodium sulphite, crystals       | do    | 90   |
| Potassium bromide               | do    | 4    |
| Sodium carbonate, crystals      | do    | 150  |
| Water to                        | ccs   | 1000 |

EDWARD BOWES KNOTT.  
GUY WILLIAM WILLIS STEVENS.

No references cited.